

# United States Patent [19]

Ikeda et al.

US005221494A

[11] Patent Number: 5,221,494  
[45] Date of Patent: Jun. 22, 1993

[54] REFRIGERANT COMPOSITION  
COMPRISING TETRAFLUOROETHANE  
REFRIGERANT AND LUBRICANT HAVING  
MISCIBILITY THEREWITH AT LOW  
TEMPERATURE

[75] Inventors: **Masanori Ikeda, Fuji; Hiroyuki Fukui, Numazu; Yoshio Suzuki, Fuji, all of Japan**

[73] Assignee: **Asahi Kasei Kogyo Kabushiki Kaisha, Osaka, Japan**

[21] Appl. No.: 582,847

[22] PCT Filed: Jun. 5, 1990

[86] PCT No.: PCT/JP90/00731

§ 371 Date: Oct. 15, 1990

§ 102(e) Date: Oct. 15, 1990

[87] PCT Pub. No.: WO90/15122

PCT Pub. Date: Dec. 13, 1990

[30] Foreign Application Priority Data

Jun. 5, 1989 [JP] Japan ..... 1-141173  
Sep. 14, 1989 [JP] Japan ..... 1-237123  
Jan. 25, 1990 [JP] Japan ..... 2-13580

[51] Int. Cl.<sup>5</sup> ..... C10M 105/54; C10M 107/38; C10N 40/30

[52] U.S. Cl. ..... 252/68; 252/54; 252/54.6; 252/67

[58] Field of Search ..... 252/67, 68, 54, 54.6; 560/180; 562/583

[56] References Cited

U.S. PATENT DOCUMENTS

3,250,807 5/1966 Fritz et al. ..... 560/180  
3,250,808 5/1966 Moore, Jr. et al. ..... 252/54.6  
3,317,484 5/1967 Fritz et al. ..... 524/881  
3,654,273 4/1972 Schuman et al. ..... 544/216  
3,660,315 5/1972 Hill et al. ..... 528/402  
3,845,051 10/1974 Zollinger ..... 544/216  
4,178,465 12/1979 Caporiccio et al. ..... 252/52 A  
4,356,291 10/1982 Darling ..... 525/403  
4,597,882 7/1986 Nishimura et al. ..... 252/51  
4,647,413 3/1987 Savu ..... 560/180  
4,755,316 7/1988 Magid et al. ..... 252/68

4,931,199 6/1990 Bierschenk et al. ..... 252/68  
5,000,864 3/1991 Strepparola et al. ..... 252/54.6

FOREIGN PATENT DOCUMENTS

51-2083 1/1976 Japan  
52-16561 2/1977 Japan  
53-5360 2/1978 Japan  
57-175185 10/1982 Japan  
60-96684 5/1985 Japan  
61-233088 10/1986 Japan  
62-146996 6/1987 Japan  
62-288692 12/1987 Japan  
1-118598 5/1989 Japan

OTHER PUBLICATIONS

Abstract of Internationales Jahrbuch der Tribologie (International Yearbook of Tribology, 1, 383-93, 1982.

Primary Examiner—Christine Skane  
Attorney, Agent, or Firm—Birch, Stewart, Kolasch & Birch

[57] ABSTRACT

A lubricant for use in a refrigeration system using a tetrafluoroethane refrigerant, which comprises a fluorine-containing compound represented by the following formula:



wherein X represents a multiple bond-containing monovalent group, and A represents a mono-, bi- or trivalent unsubstituted or partially substituted perfluorocarbon residue, a mono, bi- or trivalent unsubstituted or partially substituted perfluoroether residue or a mono-, bi- or trivalent unsubstituted or partially substituted perfluoropolyether residue.

This lubricant has a good miscibility with a tetrafluoroethane refrigerant as represented by HFC-134a over a wide range of temperatures ranging from the low temperature to the high temperature and is excellent in properties, such as heat resistance, lubricating properties, electrically insulating properties and viscosity-temperature characteristics.

5 Claims, No Drawings

**REFRIGERANT COMPOSITION COMPRISING  
TETRAFLUOROETHANE REFRIGERANT AND  
LUBRICANT HAVING MISCELLITY  
THEREWITH AT LOW TEMPERATURE**

**TECHNICAL FIELD**

The present invention relates to a refrigerant composition. More particularly, the present invention relates to a lubricant-containing refrigerant composition suitable for use in a refrigeration system employing as a refrigerant a tetrafluoroethane, preferably HFC-134a (1,1,1,2-tetrafluoroethane), which is promising as a substitute for CFC-12 (1,1-dichloro-1,1-difluoromethane) with a viewpoint of environment protection.

**BACKGROUND ART**

At present, CFC-12 is mainly used as a refrigerant for car air conditioners and refrigerators. However, development of a refrigerant which can be used as a substitution for CFC-12 has been desired with a viewpoint of protection of the ozone layer.

HFC-134a as a refrigerant has properties similar to those of CFC-12, and it can be used as a substitute for CFC-12 with only minor changes of equipment being necessary. Likewise, HFC-134 (1,1,2,2-tetrafluoroethane), which is an isomer of HFC-134a, can also be used.

In a refrigeration system using CFC-12, mineral oil is used as a lubricant for a compressor. CFC-12 is miscible with mineral oil over a wide temperature range and therefore, even in the refrigeration system where evaporation and condensation of the refrigerant are repeated, phase separation of the refrigerant from the lubricant does not occur.

However, HFC-134a is not satisfactorily miscible with mineral oil. Therefore, when mineral oil is used, the mineral oil is replaced by the refrigerant, for example, in a compressor, causing various serious problems. For example, the lubrication becomes unsatisfactory and the lubricant adheres to the inner wall of a heat exchanger, leading to a lowering of the heat exchange efficiency.

The lubricant for a refrigerator using HFC-134a as the refrigerant should be miscible with HFC-134a at least over a temperature range of from 0° to 50° C., preferably over a wide temperature range of from -20° to 70° C., more preferably over a wider temperature range of from -40° to 90° C., and most preferably over a still wider temperature range.

The lubricant should have a kinetic viscosity of from 3 to 500 centistokes (hereinafter, frequently abbreviated as "cst") at 40° C., preferably from 5 to 300 cst at 40° C., more preferably from 5 to 170 cst at 40° C., and most preferably from 10 to 150 cst at 40° C., for exerting excellent lubricating performances.

Accordingly, development of a lubricant having a desired viscosity and being miscible with HFC-134a over a wide temperature range has been desired.

Various polyoxyalkylene glycol substances have been proposed as the lubricant to be used in combination with HFC-134a. Particularly, a polyoxyalkylene glycol having at least two hydroxyl groups (specifically, polyoxypropylene glycol), disclosed in the specification of U.S. Pat. No. 4,755,316, is taught to exhibit a good miscibility with HFC-134a over a wide temperature range. However, the temperature range over which this lubricant is miscible with HFC-134a is still

unsatisfactory, and improvement of the miscibility, especially at high temperatures, is required.

Polyoxyalkylene glycols have not only unsatisfactory lubrication properties under application conditions, but also high moisture absorption properties and therefore, various problems are likely to arise with respect to, for example, the freezing of water, corrosion of metals, and lowering of the volume resistivity (such a lowering of the volume resistivity causes a problem in the case of a closed type freezer, such as a refrigerator). Accordingly, polyoxyalkylene glycols are not an excellent lubricant for a refrigeration system from a practical point of view.

A perfluoropolyether oil appears to be a lubricant miscible with HFC-134a which is a fluorine-containing compound.

Various perfluoroether oils having different structures can be mentioned. For example, there can be mentioned oils comprised mainly of recurring units, which may be either of a single type or of a plurality of types, represented by the following formula (V):



wherein n' is 1, 2 or 3 with the proviso that n' is not simultaneously 1 with respect to all of the recurring units of the perfluoroether portion.

Specific examples of perfluoroether oils include those, which are available in the market as a vacuum pump oil and a lubricating oil, having a terminal stabilized with a perfluoroalkyl group, as shown below:



and



wherein q<sub>1</sub>, q<sub>2</sub>, q<sub>3</sub>, q<sub>4</sub>, q<sub>5</sub> and q<sub>6</sub> are each a positive integer.

The present inventors examined the miscibility of these various perfluoropolyether oils with HFC-134a, and found that each oil shows a good miscibility with HFC-134a at temperatures higher than about room temperature, but oils, except those having a low molecular weight, are unsatisfactory in the miscibility with HFC-134a at low temperatures below 0° C. Accordingly, it was confirmed that these oils are not suitable as a lubricant for a refrigeration system employing HFC-134a as the refrigerant.

In Japanese Unexamined Patent Application Publication No. 60-96684, it is taught that when a fluorolubricant, such as a fluorinated silicone or a perfluoropolyether, is used in a fluorocarbon motive fluid for a heat pump, the heat resistance of a fluorocarbon refrigerant is improved. However, no description is made with respect to the miscibility of a tetrafluoroethane with a fluoro-lubricant. Japanese Unexamined Patent Application Publication No. 1-118598 teaches that a perfluoropolyether and/or a fluorinated silicone can

be used as a lubricant for fluorocarbon refrigerants. However, with respect to the miscibility at low temperatures below about room temperature, no description is made.

In Japanese Unexamined Patent Publication Application No. 62-146996, it is taught that addition of up to 5% by weight of a carboxyl group- or hydroxyl group-containing perfluoropolyether derivative as an extreme pressure additive to a lubricant is effective. However, no description is made with respect to the miscibility of this carboxyl group- or hydroxyl group-containing perfluoropolyether derivative with a fluorocarbon refrigerant, such as a tetrafluoroethane.

In Japanese Examined Patent Application Publication No. 51-2083 and the specification of U.S. Pat. No. 3,654,273, it is taught that a perfluoropolyether type triazine compound can be used as a lubricant, but no description is made with respect to the miscibility of this compound with a fluorocarbon refrigerant, such as a tetrafluoroethane. The lubricating performances of a perfluoropolyether type triazine compound and poly(hexafluoropropylene oxide) are described in Internationales Jahrbuch der Tribologie (International Yearbook of Tribology), 1, 383 (1982), but the miscibility properties of these compounds with a fluorocarbon refrigerant, such as a tetrafluoroethane, are not described at all.

In these situations, the present inventors have made researches with a view toward developing a substance showing not only a good miscibility with a tetrafluoroethane, such as HFC-134a, over a wide temperature range of from low temperatures to high temperatures, but also a viscosity ensuring satisfactory lubricating performances. As a result, it has been found that a fluorine-containing compound having a specific viscosity and having a structure represented by formula (I) defined herein or a composition comprising at least 25% by weight of this fluorine-containing compound and the balance of other oil, has not only a good miscibility with a tetrafluoroethane, such as HFC-134a but also a viscosity suitable for a lubricant for a refrigeration system and, is therefore suitable as a lubricant for use in a refrigeration system using a refrigerant comprising a tetrafluoroethane, such as HFC-134a. The present invention has now been completed, based on this finding.

It is therefore a primary object of the present invention to provide a novel lubricant for use in a refrigeration system, which exhibits not only a good miscibility with a tetrafluoroethane, such as HFC-134A which is a refrigerant promising as a substitute for CFC-12, over a wide temperature range of from low temperatures to high temperatures, but has also a viscosity suitable for a lubricant for use in a refrigeration system.

Another object of the present invention is to provide a refrigerant composition comprising the above-mentioned lubricant for use in a refrigeration system and a tetrafluoroethane refrigerant.

These and other objects, characteristic features and advantages of the present invention will become apparent from the following detailed description and the appended claims.

#### DISCLOSURE OF THE INVENTION

In accordance with the present invention, there is provided a refrigerant composition for use in a refrigeration system, comprising:

(a) a tetrafluoroethane refrigerant, and

(b) a lubricant selected from the group consisting of a fluorine-containing compound (I) and a lubricating composition comprising the compound (I) in an amount of at least 25% by weight, based on the weight of the lubricating composition,

the lubricant having a kinetic viscosity of from 3 to 500 centistokes at 40° C.,  
the compound (I) being represented by the formula:



wherein:

X is a multiple bond-containing monovalent group selected from the group consisting of:

(i) a carbonyl-containing group of the formula:



wherein Y represents a hydroxyl group, an unsubstituted or partially substituted alkoxy group having from 1 to 300 carbon atoms, an unsubstituted or partially substituted aryloxy group having from 6 to 300 carbon atoms, an unsubstituted or partially substituted alkylthio group having from 1 to 300 carbon atoms, an unsubstituted or partially substituted arylthio group having from 6 to 300 carbon atoms, an unsubstituted or partially substituted amino group having from 0 to 300 carbon atoms, an unsubstituted or partially substituted monovalent aliphatic hydrocarbon residue having from 1 to 100 carbon atoms, or an unsubstituted or partially substituted monovalent aromatic hydrocarbon residue having from 6 to 100 carbon atoms,

(ii) a nitrile group and

(iii) a triazine ring-containing group of the formula:



wherein R represents an unsubstituted or partially substituted bivalent perfluoropolyether residue having from 3 to 200 carbon atoms, an unsubstituted or partially substituted bivalent perfluoroether residue having from 2 to 60 carbon atoms, an unsubstituted or partially substituted bivalent perfluorocarbon residue having from 1 to 30 carbon atoms; Z<sub>1</sub>, Z<sub>2</sub> and Z<sub>3</sub> each independently represent an unsubstituted or partially substituted monovalent perfluoropolyether having from 3 to 200 carbon atoms, an unsubstituted or partially substituted monovalent perfluoroether residue having from 2 to 60 carbon atoms, or an unsubstituted or partially substituted monovalent perfluoroalkyl group having from 1 to 30 carbon atoms, and q is an integer of from 0 to 20;

p is an integer of from 1 to 3;

A represents an unsubstituted or partially substituted mono-, bi- or trivalent perfluorocarbon residue having from 1 to 15 carbon atoms, or an unsubstituted or partially substituted mono-, bi- or trivalent perfluoroether

residue having from 2 to 15 carbon atoms, or an unsubstituted or partially substituted mono-, bi- or trivalent perfluoropolyether having from 3 to 15 carbon atoms; 1 is an integer of from 1 to 3; 5  
m is an integer of from 0 to 80; m' is 0 or 1; and n is an integer of from 1 to 4; wherein when p and/or m is not smaller than 2, the units of  $\text{OC}_n\text{F}_{2n}$  are the same or different and are not replaced or are replaced with a unit or units of the 10 formula:



(IV)

wherein B represents a bivalent perfluorocarbon residue having from 1 to 15 carbon atoms, a bivalent perfluoroether residue having from 2 to 15 carbon atoms, or a bivalent perfluoropolyether residue having from 3 to 15 carbon atoms, and X' has the same meaning as defined for X of formula (I), with the proviso that the number of a unit or units of  $\text{OC}_n\text{F}_{2n}$  replaced by a unit or units of the formula (IV) is not greater than 30% of the total number of the units of  $\text{OC}_n\text{F}_{2n}$ ; and wherein when p is not smaller than 2, the multiple bond-containing monovalent X groups are the same or different. 20  
25

As mentioned above, the present invention has been completed, based on the novel finding that a compound comprising a fluorine-containing group and a multiple bond-containing group as indispensable constituents surprisingly shows excellent miscibility with HFC-134a and is valuable as a lubricant for use in a refrigeration system using HFC-134a as a refrigerant. 30  
35

The present invention will now be described in detail.

In the lubricant having a structure represented by formula (I), which is used in the present invention, n of the unit of  $\text{OC}_n\text{F}_{2n}$  is an integer of from 1 to 4. Specific examples of units of  $\text{OC}_n\text{F}_{2n}$  include units of 40 the following structures:



(VI-1)



(VI-2)



(VI-3)



(VI-4)



(VI-5)

and



In formula (I), the value of m representing the number of units  $\text{OC}_n\text{F}_{2n}$  depends on the value of p but is generally an integer of from 0 to 80, preferably an integer of from 0 to 60, and more preferably an integer of from 0 to 40.

In formula (I), 1 is an integer of from 1 to 3. Specific examples of units of  $\text{OC}_n\text{F}_{2n}$  include units of the following structures:



In formula (I), p is an integer of from 1 to 3.

A of formula (I) represents a mono-, bi- or trivalent perfluorocarbon residue having from 1 to 15 carbon atoms, preferably from 2 to 10 carbon atoms, a mono-, bi- or trivalent perfluoroether residue having from 2 to 15 carbon atoms, preferably from 2 to 10 carbon atoms, or a mono-, bi- or trivalent perfluoropolyether residue having from 3 to 15 carbon atoms, preferably from 3 to 10 carbon atoms.

Fluorine atoms of A can be substituted with a hydrogen atom, a chlorine atom, a bromine atom, a iodine atom or the above-mentioned multiple bond-containing monovalent group X (described in detail hereinafter), with the proviso that the number of substituted fluorine atom or atoms is not greater than 50%, preferably not greater than 30%, of the total number of fluorine atoms of unsubstituted A.

Specific examples of A include the following groups:



In the formulae described in the instant specification, Me Et and Bu represent a methyl group, an ethyl group and a butyl group, respectively.

The multiple bond-containing monovalent group X of formula (I) is a multiple bond-containing monovalent group selected from the group consisting of:

(i) a carbonyl-containing group of the formula:



(II)

wherein Y represents a hydroxyl group, an unsubstituted or partially substituted alkoxy group having from

1 to 300 carbon atoms, an unsubstituted or partially substituted aryloxy group having from 6 to 300 carbon atoms, an unsubstituted or partially substituted alkylthio group having from 1 to 300 carbon atoms, an unsubstituted or partially substituted arylthio group having from 6 to 300 carbon atoms, an unsubstituted or partially substituted amino group having from 0 to 300 carbon atoms, an unsubstituted or partially substituted monovalent aliphatic hydrocarbon residue having from 1 to 100 carbon atoms, or an unsubstituted or partially substituted monovalent aromatic hydrocarbon residue having from 6 to 100 carbon atoms,

(ii) a nitrile group and

(iii) a triazine ring-containing group of the formula:



15

20

25

30

35

wherein R represents an unsubstituted or partially substituted bivalent perfluoropolyether residue having from 3 to 200 carbon atoms, an unsubstituted or partially substituted bivalent perfluoroether residue having from 2 to 60 carbon atoms, an unsubstituted or partially substituted bivalent perfluorocarbon residue having from 1 to 30 carbon atoms; Z<sub>1</sub>, Z<sub>2</sub> and Z<sub>3</sub> each independently represent an unsubstituted or partially substituted monovalent perfluoropolyether having from 3 to 200 carbon atoms, an unsubstituted or partially substituted monovalent perfluoroether residue having from 2 to 60 carbon atoms, or an unsubstituted or partially substituted monovalent perfluoroalkyl group having from 1 to 30 carbon atoms, and q is an integer of from 0 to 20;

When p in formula (I) is 2 or 3, X groups may be the same or different.

The multiple bond-containing monovalent group X will now be described in detail.

Where Y of the carbonyl group-containing group (II) represented by formula (II) is an alkoxy group, an aryloxy group, an alkylthio group or an arylthio group, that is, where the group (II) is an ester group or a thioester group, a variety of ester groups or thioesters having different structures can be used, but preferably, groups represented by the following formula (VII) or (VII'):



(VII)

or



(VII')

are used. In formula (VII) or (VII'), R<sub>1</sub> represents a group having from 1 to 300 carbon atoms, which is selected from groups (1), (2), (3) and (4) described below.

(1) An aliphatic or aromatic group having from 1 to 30 carbon atoms, preferably from 1 to 16 carbon atoms, more preferably from 1 to 12 carbon atoms.

(2) An organic group having from 1 to 80 of, preferably from 1 to 60 of, more preferably from 1 to 40 of linkage groups selected from an ether group, an amino groups and an Si—O bond in the main chain. The molecular weight of this organic group depends on the number of ether groups, amino groups or Si—O bonds, but

the molecular weight is generally from 45 to 5,000, preferably from 45 to 3,000, more preferably 45 to 2,000. The number of carbon atoms per linkage group selected from an ether group, an amino group and an Si—O bond in the organic group is generally up to 30, preferably from 2 to 20, more preferably from 2 to 10. The number of carbon atoms of the organic group is generally from 2 to 300, preferably from 2 to 200, more preferably from 2 to 100.

The organic groups can assume various structures, examples of which include groups represented by the following formula (VII-1):



wherein D represents a hydrogen atom or an aliphatic or aromatic hydrocarbon group having from 1 to 20 carbon atoms, preferably from 1 to 10 carbon atoms, R<sub>1a</sub> represents an alkylene group having from 2 to 4 carbon atoms, R<sub>1b</sub> represents an aliphatic or aromatic hydrocarbon group having from 5 to 20 carbon atoms, R<sub>1c</sub> and R<sub>1d</sub> each represent an aliphatic or aromatic hydrocarbon group having from 1 to 10 carbon atoms, R<sub>1e</sub> represents a hydrogen atom or an aliphatic or aromatic hydrocarbon group having from 1 to 10 carbon atoms, R<sub>1f</sub> and R<sub>1g</sub> each represent an aliphatic or aromatic hydrocarbon group having from 1 to 20 carbon atoms, preferably from 1 to 15 carbon atoms, n<sub>1</sub>, n<sub>2</sub>, n<sub>3</sub> and n<sub>4</sub> each represent 0 or a positive integer, with the proviso that the sum of n<sub>1</sub>, n<sub>2</sub>, n<sub>3</sub> and n<sub>4</sub> is generally from 1 to 80, preferably from 1 to 60, more preferably from 1 to 40, and n<sub>5</sub> is 0 or 1.

(3) A group formed by substituting organic group (1) or (2) mentioned above with a substituent having up to 8 carbon atoms.

Examples of substituents having up to 8 carbon atoms include (a) an aliphatic or aromatic hydrocarbon group, (b) a polar substituent, such as a hydroxyl group, an alkoxy group, an amino group, an ester group, an amide group, a ketone group, a carboxyl group, a nitrile group or a sulfonyl group, (c) a group containing the polar substituent mentioned above, (d) a halogen atom, such as a fluorine atom, a chlorine atom or a bromine atom, and (e) a group containing the halogen atom mentioned above.

The substituted group may be a group formed by substituting a part of the hydrogen atoms of organic group (1) or (2) with the above-mentioned substituent having up to 8 carbon atoms, or a group formed by substituting the methylene groups of the main chain of organic group (1) or (2) with an ester linkage, an amide linkage, a ketone group or a sulfonyl group.

(4) A substituted group formed by substituting the hydrogen atom of the C—H bond, O—H bond or N—H bond of organic group or (1), (2) or (3) with a group represented by the following formula (VII-2):



wherein l, m, m' and n are as defined for l, m, m' and n of formula (I), and A<sub>1</sub> represents a monovalent group as defined for A of formula (I).

The number of the substituent or substituents having up to 8 carbon atoms in the substituted group (3) per one R<sub>1</sub> and the number of the substituent or substituents

of formula (VII-2) per one R<sub>1</sub> are each generally from 1 to 6, preferably from 1 to 3, more preferably 1. The number of carbon atoms of the substituted group or (3) (4) is generally from 1 to 300, preferably from 2 to 100. Examples of R<sub>1</sub> groups include the following groups:



-continued



wherein  $r_1$ ,  $r_2$ ,  $r_3$ ,  $r_4$ ,  $r_5$ ,  $r_6$ ,  $r_7$  and  $r_8$  represent a positive integer,  $l$ ,  $m$  and  $n$  are as defined for  $l$ ,  $m$  and  $n$  of formula (I), and  $\text{A}_1$  is a monovalent group as defined for  $\text{A}$  of formula (I).

Where  $\text{Y}$  is an amino group, that is, the group (II) is an amide group, a variety of groups having different structures can be used as the carbonyl-containing group represented by formula (II), preferred examples of which are those represented by the following formula (VIII):



of formula (VIII) is generally from 0 to 300, preferably from 0 to 200, more preferably from 0 to 100.

Specific examples of amide groups represented by formula (VIII) include the following groups:



wherein  $\text{R}_2$  and  $\text{R}_3$  each represent a hydrogen atom or the same substituent as  $\text{R}_1$  of formula (VII), with the proviso that  $\text{R}_2$  and  $\text{R}_3$  may be bonded together to form a cyclic structure. The number of carbon atoms in the amino group

(VIII)

60 wherein  $\text{R}_9$  and  $r_{10}$  each represent a positive integer,  $l$ ,  $m$  and  $n$  are as defined for  $l$ ,  $m$  and  $n$  of formula (I), and  $\text{A}_1$  represents a monovalent group as defined for  $\text{A}$  of formula (I).

Where  $\text{Y}$  represents an aliphatic or aromatic hydrocarbon residue, that is, the group (II) is an acyl group, the carbonyl-containing group represented by formula (II) can be, for example, a group represented by the following formula (IX):





In the above formulae,  $s_1$ ,  $s_2$  and  $s_3$  represent 0 or an integer of at least 1, which is selected so that the number of carbon atoms of  $Z_1$ ,  $Z_2$  or  $Z_3$  is from 1 to 200, preferably from 1 to 100, more from 1 to 60, and  $E$  represents a bivalent perfluorocarbon residue having from 1 to 15 carbon atoms, a bivalent perfluoropolyether residue having from 3 to 15 carbon atoms, or a bivalent perfluoroether residue having from 2 to 15 carbon atoms.

In formula (III),  $q$  is an integer of from 0 to 20, preferably from 0 to 10, more preferably from 0 to 5.

The compound of formula (I) used in the present invention can be easily synthesized from a compound which is represented by the same formula as formula (I), wherein substituent group  $X$  of formula (I) is, however, a carboxylic acid fluoride group ( $-\text{COF}$ ) [or a group  $-\text{CF}_2\text{O}^\ominus$  (which is in the state equilibrated with  $-\text{COF} + \text{F}^\ominus$ , having a reactivity equivalent to that of the carboxylic acid fluoride group], a carboxyl group or a lower alkyl ester group (hereinafter, frequently referred to as "precursor of compound (I)", according to a known process.

Examples of precursors of compound (I) and examples of processes for the synthesis thereof will now be described, although the precursors and synthesis processes are not limited to those described below.

(1) Where  $p=1$ :

A precursor represented by the following formula is used:



wherein  $\text{R}_f$  represents a perfluoroalkyl group.

Examples of compounds represented by formula (X) include an oligomer of hexafluoropropylene oxide and an oligomer of tetrafluoroethylene oxide. These compounds can be easily synthesized according to a known process.

For example, the following processes can be mentioned.

Process Disclosed in Specification of U.S. Pat. No. 3,317,484:



Process Disclosed in Journal of Macromolecular Science-Chemistry, A6(6), p. 1027 (1972):



wherein  $\text{R}_f$  represents a perfluoroalkyl group.  
Process Disclosed in European patent Publication No. 0,148,482:



45

(2) Where  $p=2$  or 3:  
A precursor represented by the following formula is used:



50

60

wherein  $\text{R}'_f$  represent a bivalent or trivalent perfluorocarbon residue.

The compound represented by formula (XI) also can be easily synthesized according to a known process.

For example, the following processes can be mentioned.

Process Disclosed in Japanese Examined Patent Publication No. 50-7054:



Process Disclosed in Specification of U.S. Pat. No. 4,113,435: 10



Process Disclosed in Journal of Organic Chemistry,  
Volume 40, p. 3271 (1975):



Process Disclosed in Specification of U.S. Pat. No.  
3,250,807:



Process Disclosed in Japanese Examined Patent Application Publication No. 53-5360:



Process Disclosed in Japanese Unexamined Patent Application Publication No. 63-265920:



18

-continued



In formulae (X-1) through (X-5) and formulae (XI-1) through (XI-6),  $t_1$  through  $t_{16}$  represent 0 or a positive integer.

15 (3) Where a perfluoropolyether structure having a pendant functional group of formula (IV) is contained:

The units of  $\langle\text{OC}_n\text{F}_{2n}\rangle$  of the compound of formula (I) used in the present invention can be substituted, in a substitution ratio of not greater than 30% based on all of these units, with unit or units represented by the following formula (IV):



wherein B represents a bivalent perfluorocarbon residue having from 1 to 15 carbon atoms, a bivalent perfluoroether residue having from 2 to 15 carbon atoms, or a bivalent perfluoropolyether residue having from 3 to 15 carbon atoms, and X' has the same meaning as defined for X of formula (I).

As examples of units of by formula (IV), there can be mentioned carbonyl group-containing units derived from groups described below, which are disclosed in Japanese Unexamined Patent Application Publication No. 57-176974 and Japanese Unexamined Patent Application Publication No. 57-176973:



and various carbonyl-containing units derived from



When  $p$  is not smaller than 2, a plurality of the multiple bond-containing monovalent  $X$  groups may be the same or different.

65 The precursors of compound (I) can be synthesized according to the processes described above. The carboxylic acid fluoride group, carboxyl group or lower alkyl ester group of the precursor can be easily con-

verted to a nitrile group, a carboxyl group, an ester group, a thioester group, an amide group or a ketone group in accordance with a known process.

Examples of this conversion reaction are described below, although employable conversion reactions are not limited to those exemplified below.



Formation of the triazine ring can be attained by treating the nitrile group according to a known process. Examples of the triazine ring-forming reaction are described below, although employable reactions are not limited to those exemplified below.



Compounds represented by formula (I), which may be employed individually or in combination, can be advantageously used as a lubricant for a refrigeration system using a refrigerant comprising a tetrafluoroethane.

Moreover, the compound of formula (I) can be used in the form of a mixture thereof with at least one oil other than the compound of formula (I).

-continued



Oils employable in combination with the compound of formula (I) are not specifically limited, and can be those which are conventionally used as lubricants. For example, there can be mentioned perfluoropolyether oils, chlorofluorocarbon oils, polyalkylene glycol oils, hydrocarbon oils, ester oils, silicone oils and fluorinated silicone oils. An appropriate oil is selected among these oils, taking into consideration the miscibility with the compound of formula (I) and the viscosity or lubrication characteristics of the lubricating composition to be obtained.

When the compound of formula (I) is used in mixture with another oil or other oils, the amount of the compound of formula (I) is determined, taking into consideration the miscibility of the lubricating composition (to be obtained) with the refrigerant and the viscosity of the lubricating composition. In order to manifest a satisfactory miscibility with a tetrafluoroethane, the compound of formula (I) is used in an amount of at least 25% by weight, preferably at least 40% by weight, more preferably at least 50% by weight, based on the total weight of the lubricating composition.

When a single compound of formula (I) is used as the lubricant for a refrigerant comprising a tetrafluoroethane, it is desired that the compound of formula (I) have a kinetic viscosity of from 3 to 500 cst at 40° C. or from 5 to 500 cst at 40° C., preferably from 5 to 170 cst at 40° C., more preferably from 10 to 150 cst at 40° C.

When the viscosity is too low, satisfactory lubrication properties cannot be obtained in a compression zone. On the other hand, when the viscosity is too high, the rotation torque of the compressor disadvantageously becomes too high.

When a mixture of two or more of compounds represented by formula (I) or a mixture of the compound of formula (I) with another oil or other oils is used, the viscosity of the compound of formula (I) per se is not particularly critical, but the mixture is required to have a viscosity within the range described above with respect to the single use of the compound of formula (I).

In the present invention, the weight ratio of the total amount of the refrigerant to the total amount of the lubricant is in the range of from 99/1 to 1/99, preferably from 99/1 to 50/50, more preferably from 99/1 to 70/30.

Additives ordinarily added to lubricants, such as rust-preventive agents and extreme pressure additives, can be added, in a conventionally employed amount, to the lubricant-containing refrigerant composition for use in a refrigeration system.

The compound represented by formula (I) has a good miscibility with HFC-134a over a wide temperature range. For example, the lower limit temperature at which a perfluoropolyether is miscible with HFC-134a is generally about 0° C. or higher, except the case where the molecular weight of the perfluoropolyether is low. In contrast, with respect to the compound represented by formula (I), the lower limit temperature at which a good miscibility with HFC-134a is exhibited can be as low as below 0° C., and compounds of formula (I) having a lower limit temperature for this miscibility of below -10° C., preferably below -20° C., more preferably below -40° C., most preferably below -78° C. can be obtained.

Furthermore, compounds of formula (I) in which the upper limit temperature for miscibility with HFC-134a is above 70° C., preferably above 80° C. or more preferably above 90° C., can be easily obtained.

Accordingly, when the compound of formula (I) or a lubricating composition comprising the compound of formula (I) is used as the lubricant in a refrigerator employing a tetrafluoroethane represented by HFC-134a, both of the defect of a conventional perfluoropolyether lubricant, namely, too high a lower limit temperature for miscibility with HFC-134a, and the defect of a conventional hydrocarbon type polyglycol lubricant, namely, too low a upper limit temperature for miscibility with HFC-134a, can be overcome.

Moreover, it has been confirmed that the compound represented by formula (I) has not only low water absorption properties but also excellent lubrication properties, which are desired properties for a lubricant.

When the compound of formula (I) is subjected to testing for stability evaluation (which is the so-called sealed tube test) wherein the compound of formula (I) is heated in the presence of HFC-134a together with a metal, such as copper, brass, aluminum or carbon steel, excellent results are obtained. Namely, the compound of formula (I) is stable even at 175° C. and the surface of the metal shows substantially no change.

Accordingly, the compound represented by formula (I) or an oil comprising this compound as the main component is useful as a lubricant for various refrigeration systems using HFC-134a as the refrigerant, such as refrigerators, freezers and car air conditioners.

Furthermore, the compound represented by formula (I) or an oil comprising this compound as the main component is also valuable as a lubricant for a refrigerator using as the refrigerant HFC-134 (1,1,2,2-tetrafluoroethane), which is an isomer of HFC-134a.

Therefore, in an other aspect of the present invention, there is provided a method for imparting lubrication properties to a tetrafluoroethane refrigerant for a refrigeration equipment, which comprises adding to the refrigerant a lubricant oil selected from the group consisting of a fluorine-containing compound (I) and a lubricating composition comprising compound (I) in an amount of at least 25% by weight, based on the lubricating composition, the compound (I) being represented by the formula:



wherein:

X is a multiple bond-containing monovalent group selected from the group consisting of:

(i) a carbonyl-containing group of the formula:



wherein Y represents a hydroxyl group, an unsubstituted or partially substituted alkoxy group having from 1 to 300 carbon atoms, an unsubstituted or partially substituted aryloxy group having from 6 to 300 carbon atoms, an unsubstituted or partially substituted alkylthio group having from 1 to 300 carbon atoms, an unsubstituted or partially substituted arylthio group having from 6 to 300 carbon atoms, an unsubstituted or partially substituted amino group having from 0 to 300 carbon atoms, an unsubstituted or partially substituted monovalent aliphatic hydrocarbon residue having from 1 to 100 carbon atoms, or an unsubstituted or partially sub-

stituted monovalent aromatic hydrocarbon residue having from 6 to 100 carbon atoms,  
(ii) a nitrile group and  
(iii) a triazine ring-containing group of the formula:



wherein R represents an unsubstituted or partially substituted bivalent perfluoropolyether residue having from 3 to 200 carbon atoms, an unsubstituted or partially substituted bivalent perfluoroether residue having from 2 to 60 carbon atoms, an unsubstituted or partially substituted bivalent perfluorocarbon residue having from 1 to 30 carbon atoms; Z<sub>1</sub>, Z<sub>2</sub> and Z<sub>3</sub> each independently represent an unsubstituted or partially substituted monovalent perfluoropolyether having from 3 to 200 carbon atoms, an unsubstituted or partially substituted monovalent perfluoroether residue having from 2 to 60 carbon atoms, or an unsubstituted or partially substituted monovalent perfluoroalkyl group having from 1 to 30 carbon atoms, and q is an integer of from 0 to 20;

p is an integer of from 1 to 3;

A represents an unsubstituted or partially substituted mono-, bi- or trivalent perfluorocarbon residue having from 1 to 15 carbon atoms, or an unsubstituted or partially substituted mono-, bi- or trivalent perfluoroether residue having from 2 to 15 carbon atoms, or an unsubstituted or partially substituted mono-, bi- or trivalent perfluoropolyether having from 3 to 15 carbon atoms;

1 is an integer of from 1 to 3;

m is an integer of from 0 to 80;

m' is 0 or 1; and

n is an integer of from 1 to 4;

wherein when p and/or m is not smaller than 2, the units of  $\text{--OC}_n\text{F}_{2n}\text{--}$  are the same or different and are not replaced or are replaced with a unit or units of the formula:



wherein B represents a bivalent perfluorocarbon residue having from 1 to 15 carbon atoms, a bivalent perfluoroether residue having from 2 to 15 carbon atoms, or a bivalent perfluoropolyether residue having from 3 to 15 carbon atoms, and X' has the same meaning as defined for X of formula (I), with the proviso that the number of unit or units of  $\text{--OC}_n\text{F}_{2n}\text{--}$  replaced by a unit or units of the formula (IV) is not greater than 30% of the total number of the units of  $\text{--OC}_n\text{F}_{2n}\text{--}$ ; and wherein when p is not smaller than 2, the multiple bond-containing monovalent X groups are the same or different.

The compound represented by formula (I) or an oil containing at least 25% by weight of this compound can also be used as a lubricant for a refrigeration system using as a refrigerant a mixture of a tetrafluoroethane and other fluoro-compound, such as a trifluoroethane (e.g., 1,1,1-trifluoroethane), for example, a mixture con-

taining at least 20 mole %, preferably at least 40 mole %, of a tetrafluoroethane.

#### BEST MODE FOR CARRYING OUT THE INVENTION

The present invention will now be described in detail with reference to the following examples that by no means limit the scope of the invention.

The number average molecular weight ( $M_{\text{Wn}}$ ) of the compound of formula (I) can be easily determined from <sup>19</sup>F-NMR spectrum or <sup>1</sup>H-NMR spectrum according to the process disclosed in Journal of Macromolecular Science-Chemistry, A8(3), p. 499 (1974) or an analogous process. When the compound of formula (I) is synthesized by linking a plurality of substances respectively having known number average molecular weights, the number average molecular weight of the compound of formula (I) can be easily calculated from the number average molecular weights of the starting substances.

The kinetic viscosity of the lubricant of the present invention can be determined by measuring the viscosity by means of a viscometer. As the viscometer to be used for determining the kinetic viscosity, there can be mentioned a capillary viscometer, such as a Ubbelohde viscometer, an Ostward viscometer or a Cannon-Fenske viscometer, a rotational viscometer, and a falling ball viscometer.

#### REFERENTIAL EXAMPLE 1

(1) In substantially the same manner as in the process for the polymerization of hexafluoropropylene oxide, disclosed in Japanese Examined Patent Publication No. 53-5360, as in the process for the purification of hexafluoropropylene oxide, disclosed in Japanese Unexamined Patent Publication No. 57-175185, and as in the process for the conversion of polymer terminals, disclosed in the specification of U.S. Pat. No. 3,317,484, hexafluoropropylene oxide was polymerized by using a polymerization initiator of the following formula:



to obtain  $R_{f0}(\text{CF}_2\text{OCs})_2$  having a number average molecular weight of about 1,500, in which  $R_{f0}$  represents a perfluoropolyether portion of formula (XI-5), which is represented by the following formula:



(2)  $R_{f0}(\text{CF}_2\text{OCs})_2$  obtained in (1) above was reacted with methanol to obtain  $R_{f0}(\text{COOCH}_3)_2$  exhibiting an absorption peak at  $1795\text{ cm}^{-1}$  in the infrared absorption spectrum and having number average molecular weight of about 1,500.

#### REFERENTIAL EXAMPLE 2

$R_{f0}(\text{COOCH}_3)_2$  having a number average molecular weight of 1,500 was contacted with ammonia gas, and the obtained terminal-amidated compound was heated with phosphorus pentoxide to obtain  $R_{f0}(\text{CN})_2$  exhibiting an absorption ascribed to the nitrile group at 2260

cm<sup>-1</sup> in the infrared absorption spectrum and having a number average molecular weight of about 1,500.

### REFERENTIAL EXAMPLE 3

$R_f(COOC_2H_5)_2$  having a number average molecular weight of 1,500 was reacted with dibutylamine to obtain  $R_f[CON(Bu)_2]_2$  exhibiting an absorption peak at 1682  $\text{cm}^{-1}$  in the infrared absorption spectrum and having a number average molecular weight of 1,500. 5

#### REFERENTIAL EXAMPLE 4

Hexafluoropropylene oxide was polymerized by using potassium fluoride as a polymerization initiator to obtain an oligomer of hexafluoropropylene oxide, and a trimer was isolated therefrom by distillation. The trimer was reacted with methanol to obtain  $R'_{fo}-COOMe$ . The obtained product was reacted with ammonia gas to obtain  $R'_{fo}-CONH_2$  exhibiting an absorption peak at  $1738\text{ cm}^{-1}$  in the infrared absorption spectrum and having a number average molecular weight of 495. 20

10 and 50 g of pyridine were then added. Reaction was performed at room temperature for 15 hours. After the reaction, F-113 and the excessive hexafluoropropylene oxide trimer were removed by an evaporator. Then, F-113 was added to the residue again to form a solution.

15 The solution was washed with distilled water two times, and the F-113 layer was recovered. Removal of the F-113 by means of an evaporator gave 295 g of a compound exhibiting a characteristic absorption at 1782  $\text{cm}^{-1}$  in the infrared absorption spectrum and having

20 the following structural formula (the number average molecular weight is 2,000):



### REFERENTIAL EXAMPLE 5

By substantially the same process as disclosed in the specification of Canadian Patent No. 960,222, substances of the following formulae were synthesized:

30 Substantially the same procedure as in Referential Example 6 was repeated except that a silicone compound of the following formula (the number average molecular weight was 1,000):



$$\text{NC}-\text{CF}_2\text{O}\left(\text{CF}_2\text{CF}_2\text{O}\right)_{11,12}\text{CF}_2\text{O}\left(\text{CF}_2\text{CF}_2\text{O}\right)_{11,12}\text{CF}_2\text{CN},$$

(the number average molecular weight is about 1,600 45)

was used instead of the polyoxypropylene glycol, to thereby obtain a compound of the following formula (the number average molecular weight is 2,000):



and  $t_{17}$  and  $t_{18}$  each represent a positive integer) and

$$\text{MeO}_2\text{C}=\text{CE}_2\text{O} \neq \text{CE}_2\text{CE}_2\text{O} \neq \text{CE}_2\text{O}=\text{CE}_2\text{CO}_2\text{Me}$$

(the number average molecular weight is about 1,670 60 and  $t_{10}$  and  $t_{20}$  each represent a positive integer).

The above dinitrile and dimethyl ester will frequently be referred to simply as " $R''_f(CN)_2$ " and " $R''_f(-COOMe)_2$ " respectively, hereinafter.

#### REFERENTIAL EXAMPLE 6

In 700 g of 1,1,2-trichloro-1,2,2-trifluoroethane (frequently abbreviated as "F-113") was dissolved 150 g of

55 REFERENTIAL EXAMPLE 8  
Substantially the same procedure as in Referential Example 6 was repeated except that bisphenol A of the following formula:



was used instead of the polyoxypropylene glycol, to thereby obtain a compound of the following formula:



## REFERENTIAL EXAMPLE 9

The terminal acid fluoride group of a trimer of hexafluoropropylene oxide, represented by the following formula:



was converted to a nitrile group via an amide group according to a customary procedure, and 47.7 g of the obtained compound of the following formula:



was heated at 100° C. in an ammonia atmosphere for 12 hours and then heated at 220° C. for 24 hours. After the

10

15

20

25

35

40

45

50

55

60

65

Then, 20 g of the reaction product was reacted with a compound of the following formula:



at 40° C. for 12 hours. The excessive amount of the compound of the following formula:



was removed under reduced pressure to obtain a reaction product comprised mainly of a diimidoylamidine compound exhibiting characteristic absorptions ascribed to the imidoylamidine groups at 1654, 1604 and 1520  $\text{cm}^{-1}$  in the infrared absorption spectrum, which is represented by the following formula:



reaction, ammonia was removed under reduced pressure to obtain 45 g of a compound (the boiling point was 121° C. under 0.11 mmHg) exhibiting an absorption peak ascribed to the triazine ring at 1556  $\text{cm}^{-1}$  in the infrared absorption spectrum, which is represented by the following formula:



Then, 30 g of this imidoylamidine was reacted at 40° C. with 30 g of a trimer of hexafluoropropylene oxide represented by the following formula:



to effect ring closure reaction and obtain a compound exhibiting an absorption ascribed to the triazine ring at 1556  $\text{cm}^{-1}$  in the infrared absorption spectrum, which is represented by the following formula (the number average molecular weight is 3,500):



## REFERENTIAL EXAMPLE 10

At -30° C., 30 g of  $\text{R}_{f0}(\text{CN})_2$  having a number average molecular weight of 1,500 was contacted with liquid ammonia to obtain a reaction product comprised mainly of a diamidine of the following formula:



## REFERENTIAL EXAMPLE 11

In an ammonia atmosphere, 23 g of dinitrile  $\text{R}_{f0}(\text{CN})_2$  having a number average molecular weight of 1,500 and 77 g of a compound of the following formula:



were heated at 100° C. for 24 hours and then at 240° C. for 100 hours. After the reaction, ammonia was removed under reduced pressure, and the residue was purified by means of a silica gel column by using perfluorohexane as a solvent. The solvent was removed under reduced pressure. Then, distillation under reduced pressure was performed to remove 43 g of a fraction (having a boiling point of 132° C. under 0.13 mmHg) composed mainly of a compound of the following formula:



to thereby obtain 46 g of an oil having a kinetic viscosity 20 of 81 cst at 40° C., which was composed mainly of a compound of the following formula:



### EXAMPLE 1

A glass tube was charged with 0.5 g of  $\text{R}_{f0}(\text{COOMe})_2$  (having a number average molecular weight 35 of about 1,500 and a kinetic viscosity of 10 cst at 40° C.) synthesized according to the process of Referential Example 1. The glass tube was cooled by liquid nitrogen. The internal pressure of the glass tube was reduced and, about 1.5 g of HFC-134a was introduced into the 40 glass tube. The glass tube was sealed and placed in a temperature-adjusted water tank. When the temperature was equilibrated, the temperature range for  $\text{R}_{f0}(\text{COOMe})_2$ 's being miscible with HFC-134a was measured according to the method in which the miscibility 45

of  $\text{R}_{f0}(\text{COOMe})_2$  with HFC-134a was judged with the naked eye. The miscibility at temperatures lower than room temperature was likewise measured while cooling the sample with methanol as a cooling medium.

As the result, it was found that the lower limit temperature for  $\text{R}_{f0}(\text{COOMe})_2$  to be miscible with HFC-134a was below -78° C. and the upper limit temperature for being miscible with HFC-134a was above 90° C.

With respect to each of the compounds of formula (I) synthesized by substantially the same methods as described in Referential Examples 1 through 11, the miscibility with HFC-134a was examined in the same manner as described in Example 1. The obtained results are shown in Table 1 together with data of the kinetic viscosity at 40° C.

### EXAMPLES 2 THROUGH 31

With respect to various compounds of formula (I) and mixtures of these compounds with a per-

fluoropolyether oil, the miscibility with HFC-134a was examined at -50° C., -10° C. and 90° C.

The obtained results are shown in Table 2.

### COMPARATIVE EXAMPLES 1 THROUGH 9

The miscibility of commercially available perfluoropolyethers and various polyalkylene glycols with HFC-134a was examined in the same manner as described in Example 1. The obtained results are shown in Tables 3 and 4 together with data of the kinetic viscosity at 40° C.

In Tables 1 through 10,  $\overline{M}_n$  means the number average molecular weight, and  $n$  and  $m_1$  through  $m_6$  each represent a positive integer.

TABLE I

| Example No. | Structural formula                                                                                                                                                                                      | $\overline{M}_n$ | Temperature range<br>for being miscible<br>with HFC-134a |                            |                            |
|-------------|---------------------------------------------------------------------------------------------------------------------------------------------------------------------------------------------------------|------------------|----------------------------------------------------------|----------------------------|----------------------------|
|             |                                                                                                                                                                                                         |                  | Kinetic<br>viscosity<br>(cst, 40° C.)                    | lower limit<br>temperature | upper limit<br>temperature |
| 1           | $R_f/\text{COOMe}_2$                                                                                                                                                                                    | 1,500            | 10                                                       | below<br>-78° C.           | above<br>90° C.            |
| 2           | "                                                                                                                                                                                                       | 2,000            | 21                                                       | below<br>-78° C.           | above<br>90° C.            |
| 3           | "                                                                                                                                                                                                       | 5,000            | 125                                                      | -78° C.<br>-20° C.         | above<br>90° C.            |
| 4           | $R_f/\text{CN}_2$                                                                                                                                                                                       | 1,500            | 10                                                       | below<br>-78° C.           | above<br>90° C.            |
| 5           | "                                                                                                                                                                                                       | 4,000            | 66                                                       | -78° C.<br>-20° C.         | above<br>90° C.            |
| 6           | $R_f/\text{COO}(\text{CH}_2\text{CH}_2\text{O})_2\text{CH}_3)_2$                                                                                                                                        | 1,500            | 10                                                       | below<br>-78° C.           | above<br>90° C.            |
| 7           | $R_f/\text{CON}(\text{Bu})_2$                                                                                                                                                                           | 1,500            | 70                                                       | below<br>-78° C.           | above<br>90° C.            |
| 8           | $R_f/\text{CONH}_2$                                                                                                                                                                                     | 1,000            | 387                                                      | -78° C.<br>-20° C.         | above<br>90° C.            |
| 9           | $R_f/\text{CON}(\text{Bu})_2$                                                                                                                                                                           | 2,500            | 61                                                       | -30° C.                    | above<br>90° C.            |
| 10          | $\text{CF}_3\text{CF}_2\text{CF}_2\text{OCFCF}_2\text{OCF}-\text{C}-\text{O}-\left(\text{CH}_3\right)_n\text{CH}_2\text{O}\right)_n\text{C}\left(\text{CF}_3\right)_2\text{CF}_2\text{CF}_2\text{CF}_3$ | 2,000            | 52                                                       | below<br>-78° C.           | above<br>90° C.            |
| 11          | "                                                                                                                                                                                                       | 3,000            | 134                                                      | below<br>-78° C.           | 83° C.                     |
| 12          | $\text{CF}_3\text{CF}_2\text{CF}_2\text{OCF}-\text{CO}-\left(\text{CH}_3\right)_n\text{CH}_2\text{O}\right)_n\text{C}\left(\text{CF}_3\right)_2\text{CF}_2\text{CF}_3$                                  | 1,700            | 41                                                       | below<br>-78° C.           | above<br>90° C.            |
| 13          | "                                                                                                                                                                                                       | 2,700            | 110                                                      | below<br>-78° C.           | 83° C.                     |
| 14          | $\text{CF}_3\text{C}\left(\text{CF}_3\right)_2\text{O}-\left(\text{CH}_3\right)_n\text{CH}_2\text{O}\right)_n\text{C}\left(\text{CF}_3\right)_2$                                                        | 1,200            | 40                                                       | below<br>-78° C.           | above<br>90° C.            |
| 15          | $\text{CF}_3\text{CF}_2\text{CF}_2\text{OCFCF}_2\text{OCF}-\text{CO}-\text{CH}_2\text{CH}_2\text{CH}_2\text{CH}_2\text{O}-\text{C}\left(\text{CF}_3\right)_2\text{CF}_2\text{CF}_3$                     | 1,600            | 50                                                       | -10° C.                    | above<br>90° C.            |

TABLE 1-continued

| Example No. | Structural formula                                                                                                                                                                                                                                                                                                                                               | $\overline{M}_n$ | Temperature range<br>for being miscible<br>with HFC-134a |                            |                            |
|-------------|------------------------------------------------------------------------------------------------------------------------------------------------------------------------------------------------------------------------------------------------------------------------------------------------------------------------------------------------------------------|------------------|----------------------------------------------------------|----------------------------|----------------------------|
|             |                                                                                                                                                                                                                                                                                                                                                                  |                  | Kinetic<br>viscosity<br>(cst, 40° C.)                    | lower limit<br>temperature | upper limit<br>temperature |
| 16          | $\begin{array}{c} \text{CF}_3 \text{ O} \\    \\ \text{CF}_3 \text{CF}_2 \text{CF}_2 \text{OCF} - \text{C} - \text{O} + \text{CH}_2 \text{CH}_2 \text{CH}_2 \text{O} \xrightarrow{n} \text{C} - \text{CFOCF}_2 \text{CF}_2 \text{CF}_3 \end{array}$                                                                                                              | 1,300            | 43                                                       | -10° C.                    | above<br>90° C.            |
| 17          | $\begin{array}{c} \text{CF}_3 \text{ O} \\    \\ \text{CF}_3 \text{CF}_2 \text{CF}_2 \text{OCF} - \text{C} \text{NH} - \text{CH}_2 \text{CH}_2 \text{CH}_2 \text{O} + \text{CH}_2 \text{CH}_2 \text{CH}_2 \text{O} \\ \text{---CH}_2 \text{CH}_2 \text{CH}_2 \text{NHC} - \text{CF} - \text{OCF}_2 \text{CF}_2 \text{OCF}_2 \text{CF}_2 \text{CF}_3 \end{array}$ | 1,700            | 257                                                      | -3° C.                     | above<br>90° C.            |
| 18          | $\begin{array}{c} \text{CF}_3 \text{ O} \\    \\ \text{CF}_3 \text{CF}_2 \text{CF}_2 \text{OCF}_2 \text{OCF} - \text{CO} + \text{CH}_2 \text{CH}_2 \text{O} \xrightarrow{n} \text{OC} - \text{CFOCF}_2 \text{CF}_2 \text{OCF}_2 \text{CF}_2 \text{CF}_3 \end{array}$                                                                                             | 2,000            | 82                                                       | below<br>-78° C.           | above<br>90° C.            |
| 19          | $\begin{array}{c} \text{CF}_3 \text{ O} \\    \\ \text{CF}_3 \text{CF}_2 \text{OCF}_2 \text{OCF} - \text{CO} + \text{CH}_2 \text{CH}_2 \text{O} \xrightarrow{n} \text{OC} - \text{CFOCF}_2 \text{CF}_2 \text{OCF}_2 \text{CF}_2 \text{CF}_3 \end{array}$                                                                                                         | 1,160            | 15                                                       | below<br>-78° C.           | above<br>90° C.            |
| 20          | $\begin{array}{c} \text{CH}_3 \text{CH}_2 \text{C} \left( \begin{array}{c} \text{CF}_3 \text{ O} \\    \\ \text{CH}_2 \text{OC} - \text{CFOCF}_2 \text{CF}_2 \text{OCF}_2 \text{CF}_2 \text{CF}_3 \end{array} \right)_3 \end{array}$                                                                                                                             | 1,570            | 30                                                       | below<br>-78° C.           | above<br>90° C.            |
| 21          | $\begin{array}{c} \text{CF}_3 \text{ O} \\    \\ \text{CF}_3 \text{CF}_2 \text{OCF}_2 \text{OCF} - \text{C} - \text{O} - \text{CH}_2 \text{CH}_2 \text{OCH}_2 \text{CH}_2 \text{CH}_2 \text{O} \\ \text{---Si} \left( \begin{array}{c} \text{CH}_3 \\   \\ \text{CH}_3 \end{array} \right)_3 \end{array}$                                                        | 2,000            | 9                                                        | below<br>-78° C.           | above<br>90° C.            |
| 22          | $\text{C}_9\text{H}_{19} \text{---} \text{C}_6\text{H}_4 \text{---} \text{OCOCF}_3$                                                                                                                                                                                                                                                                              | 316              | 6                                                        | -70° C.                    | above<br>90° C.            |

TABLE I-continued

| Example No. | Structural formula | Temperature range<br>for being miscible<br>with HFC-134a |                                       |                            |                            |
|-------------|--------------------|----------------------------------------------------------|---------------------------------------|----------------------------|----------------------------|
|             |                    | $\overline{M}_n$                                         | Kinetic<br>viscosity<br>(cst, 40° C.) | lower limit<br>temperature | upper limit<br>temperature |
| 23          |                    | 532                                                      | 11                                    | -45° C.                    | above<br>90° C.            |
| 24          |                    | 420                                                      | 39                                    | below<br>-78° C.           | above<br>90° C.            |
| 25          |                    | 852                                                      | 61                                    | below<br>-78° C.           | above<br>90° C.            |
| 26          |                    | 1,184                                                    | 81                                    | below<br>-78° C.           | above<br>90° C.            |
| 27          |                    | 9                                                        | -75° C.                               | above<br>90° C.            | above<br>90° C.            |
| 28          |                    | 24                                                       | -42° C.                               | above<br>90° C.            | above<br>90° C.            |

TABLE 1-continued

| Example No. | Structural formula                                                                                                                                                                                                                                                                                                                                                                                                                                                                                                                                                                                                                                                                                                                                                                                                                                                                             | $\overline{M}_n$ | Temperature range for being miscible with HFC-134a |                         |                         |
|-------------|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|------------------|----------------------------------------------------|-------------------------|-------------------------|
|             |                                                                                                                                                                                                                                                                                                                                                                                                                                                                                                                                                                                                                                                                                                                                                                                                                                                                                                |                  | Kinetic viscosity (cst, 40° C.)                    | lower limit temperature | upper limit temperature |
| 29          | $  \begin{array}{c}  \text{CF}_3 \quad \text{CF}_3 \\    \quad   \\  \text{CF}—\text{O}—\text{CF}_2\text{CF}—\text{OCF}_2\text{CF}_2\text{CF}_3 \\    \quad   \quad   \\  \text{CF}_3 \quad \text{CF}_3 \quad \text{CF}_3 \\    \quad   \quad   \\  \text{CFOCF}_2\text{CFOCF}_2\text{CF}_2\text{CF}_3  \end{array}  $                                                                                                                                                                                                                                                                                                                                                                                                                                                                                                                                                                         | 83               | —35° C.                                            | above 90° C.            | above 90° C.            |
| 30          | $  \begin{array}{c}  \text{CF}_3 \quad \text{CF}_3 \quad \text{CF}_3 \\    \quad   \quad   \\  \text{C}=\text{N} \quad \text{N}=\text{C} \quad \text{C}=\text{N} \\     \quad    \quad    \\  \text{CF}_3 \quad \text{N} \quad \text{CF}_3 \\    \quad   \quad   \\  \text{C}=\text{N} \quad \text{N}=\text{C} \quad \text{C}=\text{N} \\     \quad    \quad    \\  \text{R}_{f6}—\text{C} \quad \text{C} \quad \text{C}—\text{R}_{f6} \\    \quad   \quad   \\  \text{CF}_3\text{CF}_2\text{CF}_2\text{O}—\text{CFCF}_2\text{OCF}—\text{C} \quad \text{C} \quad \text{C}—\text{R}_{f6}—\text{C} \quad \text{C} \quad \text{C}—\text{R}_{f6} \\    \quad   \quad   \quad   \quad   \quad   \\  \text{CFOCF}_2\text{CFOCF}_2\text{CF}_2\text{CF}_3 \quad \text{CFOCF}_2\text{CFOCF}_2\text{CF}_2\text{CF}_3 \\    \quad   \quad   \quad   \quad   \quad   \\  \text{M}_n: 3,600  \end{array}  $ | 354              | —7° C.                                             | above 90° C.            | above 90° C.            |
| 31          | $  \begin{array}{c}  \text{R}_{f6}(\text{COOH})_2 \quad (\overline{M}_n: 1,500) \\  \text{R}_{f6}(\text{COSBu})_2 \quad (\overline{M}_n: 2,100)  \end{array}  $                                                                                                                                                                                                                                                                                                                                                                                                                                                                                                                                                                                                                                                                                                                                | 24               | below —78° C.                                      | above 90° C.            | above 90° C.            |

Note:



TABLE 2

| Exam-<br>ple<br>No. | Structural Formula  | Kinetic<br>viscosity<br>(cst. 40° C.) | Miscibility with |         |        |
|---------------------|---------------------|---------------------------------------|------------------|---------|--------|
|                     |                     |                                       | -50° C.          | -10° C. | 90° C. |
| 32                  |                     | 59                                    | ○                | ○       | ○      |
| 33                  |                     | 42                                    | ○                | ○       | ○      |
| 34                  |                     | 120                                   | ✗                | ○       | ○      |
|                     | (n ≈ 2) (Mn: 4,150) |                                       |                  |         |        |
| 35                  |                     | 40                                    | ✗                | ○       | ○      |
| 36                  |                     | 28                                    | ✗                | ○       | ○      |

TABLE 2-continued

| Exam-<br>ple<br>No. | Structural Formula | Kinetic<br>viscosity<br>(cst, 40° C.) | Miscibility with<br>HFC-134a |         |        |
|---------------------|--------------------|---------------------------------------|------------------------------|---------|--------|
|                     |                    |                                       | -50° C.                      | -10° C. | 90° C. |
| 37                  |                    | 46                                    | X                            | ○       | ○      |
| 38                  |                    | 23                                    | X                            |         |        |
| 39                  |                    | 10                                    | ○                            | ○       | ○      |
| 40                  |                    | 13                                    | ○                            | ○       | ○      |
| 41                  |                    | 18                                    | ○                            | ○       | ○      |
| 42                  |                    | 19                                    | ○                            | ○       | ○      |
| 43                  |                    | 40                                    | X                            | ○       | ○      |
| 44                  |                    | 14                                    | X                            | ○       | ○      |
| 45                  |                    | 15                                    | X                            | ○       | ○      |

Note:

○: miscible  
X: phase separation\*1: F-CF<sub>2</sub>CF<sub>2</sub>CF<sub>2</sub>O- $\overline{m}_2$  CF<sub>2</sub>CF<sub>3</sub> supplied by Daikin Kogyo, Japan

TABLE 3

| Comparative<br>Example No. | Lubricant         | Mn    | Kinetic<br>viscosity | Temperature range for being<br>miscible with HFC-134a |                            |
|----------------------------|-------------------|-------|----------------------|-------------------------------------------------------|----------------------------|
|                            |                   |       | (cst, 40° C.)        | lower limit<br>temperature                            | upper limit<br>temperature |
| 1                          | KRYTOX ® 143AY *2 | 3,000 | 50                   | 5° C.                                                 | above 90° C.               |
| 2                          | KRYTOX ® 143AX *2 | 4,800 | 134                  | 25° C.                                                | above 90° C.               |
| 3                          | DEMNUM ® S-20 *1  | 2,700 | 25                   | -5° C.                                                | above 90° C.               |
| 4                          | FOMBLIN ® M-03 *3 | 4,000 | 17                   | -5° C.                                                | above 90° C.               |
| 5                          | FOMBLIN ® Y-06 *4 | 1,800 | 27                   | -5° C.                                                | above 90° C.               |

### Notes:

\*1:  $\text{F}-\text{CF}_2\text{CF}_2\text{CF}_2\text{O}-\text{CF}_2\text{CF}_3$  supplied by Daikin Kogyo, Japan



\*2:  $\text{FCF}_2\text{O} \xrightarrow{\text{H}_2\text{O}} \text{CF}_2\text{CF}_3$  supplied by Du Pont, USA

\*3:  $\text{CF}_3\text{O} + \text{CF}_2\text{CF}_2\text{O} \rightarrow \text{CF}_2\text{O} + \text{CF}_3$  supplied by Montefluos, Italy.



\*4:  $\text{CF}_3\text{O} + \text{CF}_3\text{CF}_2\text{O} \xrightarrow{\text{heat}} \text{CF}_2\text{O} \xrightarrow{\text{heat}} \text{CF}_3$  supplied by Montefluos, Italy.

TABLE 4

| Comparative Example No. | Structural formula                                                                                           | Mn    | Kinetic viscosity | Temperature range for being miscible with HFC-134a |                         |
|-------------------------|--------------------------------------------------------------------------------------------------------------|-------|-------------------|----------------------------------------------------|-------------------------|
|                         |                                                                                                              |       | (cst, 40° C.)     | lower limit temperature                            | upper limit temperature |
| 6                       | $\begin{array}{c} \text{CH}_3 \\   \\ \text{HO} - \text{CH} - \text{CH}_2 - \text{O} - \text{H} \end{array}$ | 2,000 | 171               | -60° C.                                            | 0° C.                   |
| 7                       | "                                                                                                            | 1,000 | 82                | -78° C.                                            | 62° C.                  |
| 8                       | $\text{HO} - \text{CH}_2 - \text{CH}_2 - \text{CH}_2 - \text{CH}_2 - \text{O} - \text{H}$                    | 650   | 134               | (not miscible at 20° C.)                           |                         |
| 9                       | $\text{HO} - \text{CH}_2 - \text{CH}_2 - \text{O} - \text{H}$                                                | 1,000 | 96                | (not miscible at 20° C.)                           |                         |

#### EXAMPLES 46 THROUGH 49

#### Evaluation of Heat Resistance (Sealed Tube Test)

A glass tube was charged with 0.6 ml of  $R_f(-40$  COOMe)<sub>2</sub> (number average molecular weight = 2,000) purified by means of a silica gel column, HFC-134a and test pieces of iron, copper and aluminum, and the glass tube was then sealed to obtain a test sample. The test sample was heated at 175° C. for 10 days. After the 45 heating, any change of the hue of the test sample and any change of the surfaces of the metal pieces were

examined. It was found that the hue of the test sample and the surfaces of the metals were not changed. Furthermore, the viscosity and infrared absorption spectrum of  $R_6(COOME)_2$  were not changed.

The heat resistances of various compounds of the present invention were evaluated according to the sealed tube test in the same manner as described above. The obtained results are shown in Table 5. It was found that the compounds of the present invention have a satisfactorily high heat resistance.

TABLE 5

TABLE 5-continued

## EXAMPLES 50 THROUGH 54

Use was made of a Falex tester. Under conditions such that the oil temperature at the start of the testing was adjusted at 20° C. and a load of 300 pounds was applied, the tester was driven for 3 minutes. While increasing the load, 100 pounds by 100 pounds, the tester was driven for 1 minute under each load until seizing was caused. The measurement of the seizing loads of various compounds of the present invention was con-

20 ducted. The results are shown in Table 6. It was found that each of the compounds has excellent lubrication properties.

## COMPARATIVE EXAMPLES 10 THROUGH 13

25 The seizing loads of commercially available per-fluoropolyether oils, polyoxyalkylene glycols and mineral oils were measured in the same manner as described in Example 50. The obtained results are shown in Table 7.

TABLE 6

| Example No. | Structural formula                             | Kinetic viscosity (cst, 40° C.) | Seizing load (pounds) |
|-------------|------------------------------------------------|---------------------------------|-----------------------|
| 50          | $R_{f_0}(COOMe)_2$ ( $\overline{M_n}$ : 5,000) | 125                             | above 1,500           |
| 51          | $R'_{f_0}-COOMe$ ( $M_n$ : 1,500)              | 10                              | above 1,500           |
| 52          |                                                | 41                              | 700                   |
| 53          |                                                | 9                               | above 1,500           |
| 54          |                                                | 83                              | 1,300                 |

TABLE 7

| Comparative Example No. | Lubricant                                                                                                                                                    | Kinetic viscosity (cst, 40° C.) | Seizing load (pounds) |
|-------------------------|--------------------------------------------------------------------------------------------------------------------------------------------------------------|---------------------------------|-----------------------|
| 10                      | DEMNUM ® S-65 *5                                                                                                                                             | 65                              | above 1,500           |
| 11                      | $  \begin{array}{c}  \text{CH}_3 \\    \\  \text{H} - \left( \text{O} - \text{CH}_2 \text{CH} \right)_n \text{OH} \\    \\  \text{Mn: 1,000}  \end{array}  $ | 73                              | 700                   |
| 12                      | SUNISO ® 3GS *6                                                                                                                                              | 30                              | 500                   |
| 13                      | SUNISO ® 5GS *7                                                                                                                                              | 97                              | 400                   |

**Note:**

\*5:  $\text{F}-\text{CF}_2\text{CF}_2\text{CF}_2\text{O}-\text{CF}_2\text{CF}_3$  supplied by Daikin Kogyo, Japan

\*6: naphthalene type mineral oil supplied by Nippon San Sekiyu, Japan

\*7: naphthalene type mineral oil supplied by Nippon San Sekiyu, Japan

**EXAMPLES 55 AND 56 AND COMPARATIVE 20  
EXAMPLES 14 AND 15**

### Breakdown Voltage

According to the method of JIS C2101 (test method for electrically insulating oils), the breakdown voltages of various compounds of the present invention and polypropylene glycols were measured. The obtained results are shown in Table 8. It was found that each of the compounds of the present invention has a satisfactorily high breakdown voltage.

EXAMPLES 57 THROUGH 59 AND  
COMPARATIVE EXAMPLES 16 AND 17

## Water Absorption Properties

Various compounds of the present invention, poly-  
25 propylene glycols and mineral oils were allowed to stand in a constant-temperature and constant-humidity vessel maintained at a temperature of 40° C. and at a relative humidity of 80%, and the equilibrium water absorptions were measured. The obtained results are shown in Table 9. It was found that the compound of

TABLE 8

**Note:**

\*6: naphthene type mineral oil supplied by Nippon San Sekiyu, Japan

formula (I) according to the present invention has low water absorbing properties and is suitable as a lubricant.

TABLE 9

| Lubricant          | Equilibrated<br>water absorption |
|--------------------|----------------------------------|
| <u>Example No.</u> |                                  |
| 57                 | $R_{f0}(CN)_2$ (Mn: 4,000)       |
| 58                 | $R_{f0}(COOMe)_2$ (Mn: 5,000)    |
|                    | lower than 50 ppm                |
|                    | lower than 50 ppm                |

TABLE 9-continued

| Example No.                | Lubricant                                                                                                                                                                                                                                                                                                                                                                                                                                                                                                                                                                                                                                                                              | Equilibrated water absorption |
|----------------------------|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-------------------------------|
|                            |                                                                                                                                                                                                                                                                                                                                                                                                                                                                                                                                                                                                                                                                                        | lower than 50 ppm             |
| 59                         | $  \begin{array}{c}  \text{CF}_3 \quad \text{CF}_3 \\    \quad   \\  \text{CF}_3\text{CF}_2\text{CF}_2\text{OCFCF}_2\text{OCF} \\    \quad   \\  \text{CF}_3 \quad \text{CF}_3 \\  \text{CF}_3\text{CF}_2\text{CF}_2\text{OCFCF}_2\text{OCF} \\    \quad   \\  \text{CF}_3 \quad \text{CF}_3 \\  \text{N} \quad \text{N} \\     \quad    \\  \text{C}=\text{N} \quad \text{C}=\text{N} \\    \quad   \\  \text{C}-\text{R}_{f_0}-\text{C} \\    \quad   \\  \text{N} \quad \text{N} \\     \quad    \\  \text{C}=\text{N} \quad \text{C}=\text{N} \\    \quad   \\  \text{CFOCF}_2\text{CFOCF}_2\text{CF}_2\text{CF}_3 \\    \quad   \\  \text{CF}_3 \quad \text{CF}_3  \end{array}  $ |                               |
| Comparative Example No. 16 | $  \begin{array}{c}  \text{CH}_3 \\    \\  \text{H}-\left(\text{OCH}_2\text{CH}-\right)_n\text{OH} \quad (\text{Mn: 2,000})  \end{array}  $                                                                                                                                                                                                                                                                                                                                                                                                                                                                                                                                            | 40,000 ppm                    |
| 17                         | SUNISO ® 5GS *7                                                                                                                                                                                                                                                                                                                                                                                                                                                                                                                                                                                                                                                                        | 100 ppm                       |

Note:  
\*7: naphthene type mineral oil supplied by Nippon San Sekiyu, Japan

### EXAMPLES 60 AND 61 AND COMPARATIVE EXAMPLE 18

#### Viscosity (versus temperature)

The kinetic viscosities of various compounds of the present invention at 40° C. and 100° C. were measured. The obtained results are shown in Table 10 together with the data obtained with respect to a mineral oil.

It was found that in the compound of formula (I) to be used in the present invention, the difference between the viscosities at 100° C. and 40° C. is very small and the viscosity-temperature characteristics are good.

ties, electrical insulation properties and viscosity-temperature characteristics and can be used as an excellent lubricant for a refrigeration system.

We claim:

1. A method for imparting lubrication properties to a tetrafluoroethane refrigerant for refrigeration equipment, which comprises adding to said refrigerant a lubricant oil which is miscible at temperatures below -10° C. selected from the group consisting of a fluorine-containing compound (I) and a lubricating composition comprising said compound (I) in an amount of at least 25% by weight, based on said lubricating composi-

TABLE 10

| Example No.                | Lubricant                                                                                                                                                                                                                                                                                                                                                                                                                                                                                                                                                                                                                                                                              | Kinetic viscosity (cst) |         | Viscosity ratio 40° C./100° C. |
|----------------------------|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-------------------------|---------|--------------------------------|
|                            |                                                                                                                                                                                                                                                                                                                                                                                                                                                                                                                                                                                                                                                                                        | 40° C.                  | 100° C. |                                |
| 60                         | $  \begin{array}{c}  \text{CF}_3 \quad \text{CF}_3 \\    \quad   \\  \text{CF}_3\text{CF}_2\text{CF}_2\text{OCFCF}_2\text{OCF} \\    \quad   \\  \text{CF}_3 \quad \text{CF}_3 \\  \text{CF}_3\text{CF}_2\text{CF}_2\text{OCFCF}_2\text{OCF} \\    \quad   \\  \text{CF}_3 \quad \text{CF}_3 \\  \text{N} \quad \text{N} \\     \quad    \\  \text{C}=\text{N} \quad \text{C}=\text{N} \\    \quad   \\  \text{C}-\text{R}_{f_0}-\text{C} \\    \quad   \\  \text{N} \quad \text{N} \\     \quad    \\  \text{C}=\text{N} \quad \text{C}=\text{N} \\    \quad   \\  \text{CFOCF}_2\text{CFOCF}_2\text{CF}_2\text{CF}_3 \\    \quad   \\  \text{CF}_3 \quad \text{CF}_3  \end{array}  $ | 81                      | 8.7     | 0.107                          |
| 61                         | $  \begin{array}{c}  \text{CF}_3 \\    \\  \text{CF}_3\text{CF}_2\text{CF}_2\text{OCFCO} \\    \\  \text{O} \\  \text{CH}_3 \\    \\  \text{CHCH}_2\text{O} \\    \\  \text{O} \\  \text{OC} \\    \\  \text{CF}_3  \end{array}  \quad (\text{Mn: 2,300})  $                                                                                                                                                                                                                                                                                                                                                                                                                           | 78                      | 14      | 0.178                          |
| Comparative Example No. 18 | SUNISO ® 5GS *7                                                                                                                                                                                                                                                                                                                                                                                                                                                                                                                                                                                                                                                                        | 97                      | 8       | 0.083                          |

Note:  
\*7: naphthene type mineral oil supplied by Nippon San Sekiyu, Japan

### INDUSTRIAL APPLICABILITY

When a compound containing a fluorine-containing group and a multiple bond-containing group as indispensable constituents is used as a lubricant for a refrigeration system in accordance with the present invention, the lubricant exhibits a good miscibility with a tetrafluoroethane refrigerant, as represented by HFC-134a, over a wide temperature range of from low temperatures to high temperatures, and the compound has a viscosity suitable for a lubricant. Moreover, this lubricant has excellent heat resistance, lubrication proper-

ties, electrical insulation properties and viscosity-temperature characteristics and can be used as an excellent lubricant for a refrigeration system.



60 wherein:

X is a multiple bond-containing monovalent group selected from:

(i) a carbonyl-containing group of the formula:



wherein Y represents a hydroxyl group, an unsubstituted or partially substituted alkoxy group having from 1 to 300 carbon atoms, an unsubstituted or partially substituted aryloxy group having from 6 to 300 carbon atoms, an unsubstituted or partially substituted alkylthio group having from 1 to 300 carbon atoms, an unsubstituted or partially substituted arylthio group having from 6 to 300 carbon atoms, an unsubstituted or partially substituted amino group having from 0 to 300 carbon atoms, an unsubstituted or partially substituted monovalent aliphatic hydrocarbon residue having from 1 to 100 carbon atoms, or an unsubstituted or partially substituted monovalent aromatic hydrocarbon residue having from 6 to 100 carbon atoms;

p is an integer of from 1 to 3;

A represents an unsubstituted or partially substituted mono-, bi- or trivalent perfluorocarbon residue having from 1 to 15 carbon atoms, or an unsubstituted or partially substituted mono-, bi- or trivalent perfluoroether residue having from 2 to 15 carbon atoms, or an unsubstituted or partially substituted mono-, bi- or trivalent perfluoropolyether having from 3 to 15 carbon atoms;

1 is an integer of from 1 to 3;

m is an integer of from 0 to 80;

m' is 0 or 1; and

n is an integer of from 1 to 4;

wherein when said p and/or said m is not smaller than 2, the units of (OC<sub>n</sub>F<sub>2n</sub>) are the same or different and are not replaced or are replaced with a unit or units of the formula:



wherein B represents a bivalent perfluorocarbon residue having from 1 to 15 carbon atoms, a bivalent perfluoroether residue having from 2 to 15 carbon atoms, or a bivalent perfluoropolyether residue having from 3 to 15 carbon atoms,

10 and X' has the same meaning as defined for X of formula (I), with the proviso that the number of unit or units of (OC<sub>n</sub>F<sub>2n</sub>) replaced by a unit or units of the formula (IV) is not greater than 30% of the total number of said units of (OC<sub>n</sub>F<sub>2n</sub>); and wherein when said p is not smaller than 2, said multiple bond-containing monovalent X group is the same or different.

15 2. The method according to claim 1, wherein said tetrafluoroethane is 1,1,1,2-tetrafluoroethane.

20 3. The method according to claim 1, wherein the partially substituted perfluorocarbon, perfluoroether or perfluoropolyether residue of A of formula (I) is substituted with a hydrogen atom, a chlorine atom, a bromine atom, a iodine atom or a group as defined as said multiple bond-containing monovalent X group, with the proviso that the number of substituted fluorine atom or atoms is not greater than 50% of the total number of fluorine atoms of each respective unsubstituted perfluorocarbon, perfluoroether or perfluoropolyether residue.

25 30 4. The method according to any one of claims 1, 2 and 3, wherein the weight ratio of said refrigerant to said lubricant oil is 99/1 to 1/99.

35 5. The refrigerant composition according to claim 1, wherein said tetrafluoroethane is 1,1,2,2-tetrafluoroethane.

\* \* \* \* \*